

**United States Patent** [19]  
**Kullman et al.**

[11] **3,768,969**

[45] **Oct. 30, 1973**

[54] **SENSITIZED TEXTILES WITH DECREASED FORMALDEHYDE ODOR**

[75] Inventors: **Russel M. H. Kullman, Metairie; Robert M. Reinhardt, New Orleans, both of La.**

[73] Assignee: **The United States of America as represented by the Secretary of Agriculture, Washington, D.C.**

[22] Filed: **Dec. 21, 1971**

[21] Appl. No.: **210,572**

[52] U.S. Cl. .... **8/186, 8/187, 117/119.8, 117/139.4, 117/143 A**

[51] Int. Cl. .... **D06m 13/12**

[58] Field of Search .... **117/139.4, 143 A, 117/145, 119.8; 8/115.6, 116.3, 186**

[56] **References Cited**

**UNITED STATES PATENTS**

2,731,364 1/1956 Reibnitz et al. .... 117/143 A  
3,100,159 8/1963 Ullman ..... 117/139.4 X

|           |         |                                   |
|-----------|---------|-----------------------------------|
| 3,116,967 | 1/1964  | Goldstein et al. .... 117/139.4 X |
| 3,144,299 | 8/1964  | Frick et al. .... 8/116.3         |
| 3,420,702 | 1/1969  | Spangler ..... 117/139.4          |
| 3,445,279 | 5/1969  | Abrahams et al. .... 117/143 A    |
| 3,617,198 | 11/1971 | Reid et al. .... 117/139.4 X      |
| 3,666,400 | 5/1972  | Lofton et al. .... 117/139.4 X    |
| 2,859,136 | 11/1958 | Marsh et al. .... 117/139.4 X     |
| 3,546,006 | 12/1970 | Verburg et al. .... 117/139.4 X   |

*Primary Examiner—Murray Katz*

*Assistant Examiner—Theodore G. Davis*

*Attorney—R. Hoffman et al.*

[57] **ABSTRACT**

Superheated steam is utilized both to dry and remove free formaldehyde in a combined operation from textiles suitably impregnated with finishing agent and catalyst, thereby to produce a sensitized fabric with a formaldehyde odor which is imperceptible to response of the olfactory capacity of humans. The sensitized fabric of this invention can be used in the conventional post-cure process to yield durable press products.

**12 Claims, 1 Drawing Figure**



## SENSITIZED TEXTILES WITH DECREASED FORMALDEHYDE ODOR

A non-exclusive, irrevocable, royalty-free license in the invention herein described, throughout the world for all purposes of the United States Government, with the power to grant sublicenses for such purposes, is hereby granted to the Government of the United States of America.

### FIELD TO WHICH THIS INVENTION RELATES

This invention relates to a method of producing sensitized fabric with decreased formaldehyde odor for post-cure durable press products. Specifically, this invention relates to a method wherein sensitized fabrics are produced with low formaldehyde odor (imperceptible to human olfactory response) in a one step operation by use of superheated steam.

### DEFINITIONS

By sensitized fabric we mean the use of the term as employed in the textile finishing and garment fabrication industries. A sensitized fabric is one that (1) has been impregnated with a finishing agent, usually a methylol amide type crosslinking agent, capable of producing durable-press properties in cotton or cotton containing textiles and an agent capable of catalyzing the reaction between the finishing agent and the textile material, and (2) has been dried under conditions that do not cause any appreciable reaction between the finishing agent and the textile material. The sensitized fabric is then ready for use in the post-cure durable-press process. The sensitized fabric is packaged and may be stored for prolonged periods before garment manufacture in which it is cut to pattern, sewn, trimmed, then shaped by pressing to introduce creases, pleats, etc., and to smooth the garment in its final configuration. The sensitized fabric in the form of the shaped garment is then cured, usually in an oven, to affect reaction of the finishing agent and the textile material of the garment to make the shape or configuration durable to 40 wearing and laundering.

*Post-cure* processing refers to that class of finishing treatments which impart durable press properties to the textile product through a postponed cure of the sensitized cloth after the textile product has been made up into a garment or other apparel or household item. The term is widely used in the textile industry; however, the terms deferred cure and delayed cure also have been applied to this type of durable press process.

*Free formaldehyde* is the formaldehyde that is unreacted and is therefore free to volatilize from the sensitized fabric. The release of free formaldehyde can cause objectionable response, i.e., lachrymatory and sometimes allergenic, from those who come into proximity of the material. Determinations of free formaldehyde on textiles and formaldehyde release are means used to quantify formaldehyde odor.

*Superheated steam* is steam at a temperature above the temperature at which steam and water are in equilibrium at that pressure. At normal atmospheric pressure this would be steam above 212° F.

### THE PROBLEM

In the manufacture of post-cure durable-press garments a serious problem is the odor of formaldehyde from sensitized fabric which causes discomfort and sometimes is an actual health hazard to those who cut,

sew, and press the garments. When the packages of sensitized material are opened at the garment cutting plant, free formaldehyde is slowly released to create unpleasant and potentially unsafe working conditions. The free formaldehyde is due to (a) residual or unreacted formaldehyde which was present in the finishing solution when it was dried on the fabric or (b) to formaldehyde which has been produced due to demethylation of the methylolated amide compound used in finishing. Finishers would like to reduce the formaldehyde release of sensitized fabrics and to use agents which are suitable and have other desirable qualities but which are unusable because of formaldehyde release problems.

15 Among agents that could be utilized advantageously in the post-cure process, if formaldehyde release could be eliminated or reduced to an unobjectionable level, are the methylol carbamates. Fabric sensitized with methylolated carbamate agents can be particularly troublesome because of the presence of relatively high concentrations of free formaldehyde. A primary source of free formaldehyde on the sensitized fabric is the excess formaldehyde which is generally used in preparation of the finishing agent to maximize conversion of the carbamate to the dimethylol derivative.

### THE PRIOR ART

In the prior art means have been proposed for reducing free formaldehyde of finishing agents through lowering the amount of formaldehyde in preparation of the finishing agent and through reaction of the finishing agent solution with other chemicals to bind the free formaldehyde. These chemical methods have led to undesirable collateral effects on finished fabric such as decreased chlorine resistance of the finish. A process employing steam has also been used to reduce free formaldehyde on conventionally sensitized fabric.

30 Steaming has been a useful technique to achieve other objectives and is described by many workers in the textile field. It is widely used in textile dyeing and printing. Resin fixation to prevent fiber collapse has been accomplished through steaming as a means of improving abrasion resistance of fabric. Implicit to all resin fixation processes with steam is a combination of a resin builder and crosslinking agent. Curing and critical moisture levels (above 10 percent moisture content) of fabric subjected to steaming processes are required.

45 We have unexpectedly found, however, that steaming with superheated steam can be employed in a one-step operation to affect simultaneous sensitization and free formaldehyde removal.

### OBJECT OF THE INVENTION

50 It is an object of the instant invention to provide a new and improved method for producing sensitized fabrics with decreased formaldehyde odor that may be used in post-cure finishing without adverse effect on the processing and without inducing undesirable side effects that impair utility, esthetics, value, or durability of the resulting durable press products.

### HOW THE OBJECTIVE IS ACHIEVED

55 The objective is achieved by simultaneously sensitizing and reducing odor of fabric impregnated with a formaldehyde-containing formulation or formaldehyde-derivative-containing formulation through exposure

to superheated steam. Steaming thus reduces moisture content of the web fabric while releasing and carrying away free formaldehyde. Steam sensitization thus sensitizes the fabric and reduces free formaldehyde without the necessity (1) of presensitization prior to formaldehyde removal, (2) of any change in the preparation of the finishing agent, (3) of additional reaction of the finishing agent solution with other chemical agents, (4) of any fixation of a resin former to prevent fiber collapse, (5) of an additional drying step after steaming, or (6) of any other modification of the conventional post-cure durable press process. Because of the absence of such changes and modifications, steaming accomplishes the objective of sensitization and formaldehyde odor reduction without effect on the desirable characteristics of the finish and without introducing additional undesirable characteristics.

Our investigations have revealed that fabric may be dried sufficiently to effect sensitization and removal of free formaldehyde during the process of steaming with superheated steam. We have found that the steaming time must be determined for the steam temperature employed in the process to achieve drying or sensitization such that the resultant sensitized fabric has moisture contents of from about 10 percent to a lesser moisture content of about three percent. The temperature of the steam employed in the process may be varied depending on equipment available to an operator. The efficacy of steaming is a function of steam temperature. Thus, the higher the steam temperature employed the more rapid is the lowering of the moisture content of the fabric and removal of free formaldehyde.

Although our preferred embodiments are illustrated by the examples; it is also feasible to operate on either side of the preferred figure; for example, we have found that a range of about from five to 20 percent of the weight of the crosslinking agent in the formulation, and of about 0.3 to three percent of the weight of catalyst selected from Lewis Acid type catalysts normally employed in durable press finishing operations, can be useful.

#### SUMMARY OF THE INVENTION

The instant invention can be described as a method which provides a means of achieving a sensitized fabric with low free formaldehyde content, said fabric that is intended for post-cure processes (where cure is postponed until the desired configuration has been established in the sensitized fabric) to yield durable press textile products. The said method consists of subjecting fabric impregnated with a crosslinking agent and catalyst to superheated steam for selected periods of time such that the steam removes moisture and formaldehyde odor simultaneously and results in a sensitized fabric. The sensitized fabric produced by the method of this invention may be used in the post-cure durable press process without additional modifications to yield a durable press product without introduction of undesirable effects.

The detailed description and specific examples that follow are provided merely to illustrate the invention as well as preferred embodiments. These illustrations should not be construed as limiting the scope of the instant invention in any manner whatever. Numerous changes and modifications within the spirit of the invention will become apparent to those skilled in the art.

#### EXAMPLE 1

A cotton fabric was passed into and through a solution containing 10 percent (wt/wt) dimethylol methyl carbamate and 0.6 percent (wt/wt) zinc nitrate hexahydrate, the excess squeezed off, and the process was repeated to ensure thorough impregnation. A portion of the wet, impregnated fabric was sensitized by drying in an oven at 140° F for 7 minutes. Another portion of the wet impregnated fabric was sensitized by passing the fabric through a flash ager supplied with steam for a dwell time of 5.6 minutes. The steam was superheated to 240° F and circulated by mechanical convection in the flash ager. A portion of each fabric, after sensitization, was immediately analyzed for free formaldehyde content by the procedure of Reid, Reinhardt, and Bruno (American Dyestuff Reporter 54, No. 13, 54-60 [1965]). These values are listed in the table as "% FF." A second portion of each sensitized fabric, immediately after sensitization, was placed in a glass jar containing 50 ml of distilled water and sealed. The jar was placed in an oven at 120° F (49° C) for 20 hours as specified in the AATCC Test Method 112-1968 and the formaldehyde release subsequently determined. These values are listed in the table as "% HCHO Released." A third portion of each sensitized portion, immediately after sensitization, was washed, dried, and then analyzed for nitrogen content by the Kjeldahl method. A fourth portion of each sensitized fabric was subsequently cured by placing in an oven for 3 minutes at 320° F, then washed and dried.

In Table I are results of fabrics that were sensitized:

TABLE I

| Sensitization Method | Time and Temperature of Sensitization | % FF | % HCHO Released | % N <sup>1</sup> |
|----------------------|---------------------------------------|------|-----------------|------------------|
| Oven <sup>2</sup>    | 7 min./140° F                         | 0.20 | 0.66            | 0.03             |
| Steam <sup>3</sup>   | 5.6 min./240° F                       | 0.00 | 0.09            | 0.04             |

<sup>1</sup>Determined after sample was washed

<sup>2</sup>Conventional method

<sup>3</sup>New method

In Table II are results of fabrics that were cured after sensitization:

TABLE II

| Sensitization Method | % N  | WRA, W+F Deg. | Brk. Str. W, lb. | Str. Retention in Chlorination-Scorch test, % |
|----------------------|------|---------------|------------------|-----------------------------------------------|
| Oven                 | 0.56 | 276           | 36.6             | 99                                            |
| Steam                | 0.61 | 255           | 40.6             | 99                                            |
| Untreated            | —    | 191           | 48.7             | 99                                            |

The remarkable reduction in free formaldehyde and formaldehyde release due to steam sensitization is illustrated in Table I. The nitrogen values show that fixed reagent is not a necessity in the steaming process. The substantial improvement in wrinkle recovery (determined by the procedure of AATCC Test Method 66-1968 and listed in the table as WRA) over the untreated fabric obtained on curing the steam sensitized fabric illustrates that steaming is effective in sensitization. Further, there is no loss in resistance to chlorine damage (determined by the chlorination-scorch procedure of AATCC Test Method 92-1967) nor in breaking strength (ASTM D1682-64) as compared to the conventional oven sensitization. This shows that the new process is as amenable to durable press processing as the conventional method using oven sensitization.

## EXAMPLE 2

A cotton fabric was impregnated with a solution identical to that in Example 1. Portions of the wet, impregnated fabric were steam sensitized for different dwell times and steam temperatures. Portions of each sensitized fabric were analyzed for free formaldehyde content and formaldehyde release as in AATCC Test Method 112-1968 and the results appear in Table III.

TABLE III

| Time and Temperature of sensitization | % FF | % HCHO Released |
|---------------------------------------|------|-----------------|
| 8.3 min./240°F steam                  | 0.00 | 0.09            |
| 2.4 min./280°F steam                  | 0.00 | 0.15            |
| 3.7 min./280°F steam                  | 0.00 | 0.12            |
| 5.5 min./280°F steam                  | 0.00 | 0.11            |
| 7 min./140°F oven                     | 0.20 | 0.66            |

This illustrates that the new process is operative under conditions varying from about 2 minutes to about 8 minutes at steam temperatures from about 240° F to about 280° F. The remarkable reduction of formaldehyde odor is readily seen in the free formaldehyde and formaldehyde release determinations.

Other portions of each fabric, after sensitization, were subsequently post-cured in an oven for 3 minutes at 320° F then washed and dried. Evaluation of these fabrics is shown in Table IV.

TABLE IV

| Time & Temperature of sensitization | WRA<br>% N | W+F<br>deg. | Brk.<br>Str.<br>W, lb. | Str. Retention<br>in chlorination-<br>Scorch Test, % |
|-------------------------------------|------------|-------------|------------------------|------------------------------------------------------|
| 8.3 min./240°F steam                | 0.56       | 257         | 41.7                   | 94                                                   |
| 2.4 min./280°F steam                | 0.65       | 258         | 41.3                   | 100                                                  |
| 3.7 min./280°F steam                | 0.61       | 267         | 43.3                   | 100                                                  |
| 5.5 min./280°F steam                | 0.61       | 249         | 42.0                   | 92                                                   |
| Untreated                           | —          | 191         | 48.7                   | 99                                                   |

These results clearly show that improvement in wrinkle recovery angles required in post curing of sensitized fabrics to develop durable press properties is achieved using the new process.

## EXAMPLE 3

A fabric was impregnated by padding as in Example 1 using the same components in the treating bath. A portion of the wet, impregnated fabric was sensitized by drying in an oven at 140° F for 7 minutes. Another portion of the wet, impregnated fabric was steam sensitized at 280° F for 3.8 minutes and no formaldehyde odor was noted on this sensitized fabric. The oven sensitized sample and the steam sensitized sample were creased on a steam press and then post cured in an oven at 320° F for 3 minutes. After washing and tumble drying both samples had very sharp durable creases. This further illustrates that steam sensitization is as effective as oven sensitization for preparation of sensitized fabric suitable for creasing and curing to give durable press products by the post cure process.

## EXAMPLE 4

Four solutions were prepared with the following finishing agents:

Solution I dimethylol dihydroxyethyleneurea — (DMDHEU)

Solution II dimethylol ethyleneurea — (DMEU)

Solution III dimethylol 4-methoxy-5,5-dimethylpropyleneurea — (modif. PU)

Solution IV bis-methoxymethyl uron — (uron) Each solution contained 10% (wt/wt) of finishing agent with 0.6% (wt/wt) zinc nitrate hexahydrate catalyst. Four swatches of cotton printcloth were impregnated by padding as in Example 1. The four fabrics were then steam sensitized at 280° F for 3.6 minutes. A portion from each sensitized fabric was analyzed for free formaldehyde as in Example 1 and results are shown in Table V:

10

TABLE V

|    | Finishing Agent Used | % FF in Steam Sensitized Fabric |
|----|----------------------|---------------------------------|
| 15 | DMDHEU               | 0.01                            |
|    | DMEU                 | 0.01                            |
|    | Modif. PU            | 0.05                            |
|    | Uron                 | 0.04                            |

These results show a remarkably low amount of free formaldehyde in the steam sensitized fabrics.

A remaining portion of each steam sensitized fabric was creased on a steam press and then post-cured in an oven at 320° F for 3 minutes. After washing and tumbling drying, properties of the finished fabrics were evaluated, Table VI. Durable press appearance after tumble drying was determined using the AATCC three-Dimensional Durable Press Replicas described in AATCC Test Method 124-1969. Crease appearance was determined using the photographic standards of AATCC Test Method 88C-1969.

30

TABLE VI

|    | Finishing Agent Used | DP Appearance | Crease Appearance | WRA, W+F deg. |
|----|----------------------|---------------|-------------------|---------------|
| 35 | DMDHEU               | 4.5           | 5                 | 275           |
|    | DMEU                 | 2.0           | 2                 | 182           |
|    | Modif. PU            | 4.5           | 5                 | 251           |
|    | Uron                 | 4.5           | 5                 | 262           |

These results show that the new sensitization method is effective for preparation of durable press products by the post cure process with selected finishing agents. It is not effective with DMEU.

## EXAMPLE 5

A cotton printcloth was impregnated by padding to about 96 percent wet pickup of water (49 percent moisture content) and then passed for various dwell times through steam at 240° and 280° F. Actual moisture contents of the steamed fabrics were determined and are shown in the Figure.

This demonstrates that steaming was sufficient to dry wet fabrics to moisture levels suitable for use in sensitizing fabric.

We claim:

1. A method of sensitizing a cellulosic textile for use in the preparation of a post-cure durable-press product while simultaneously rendering the textile free of formaldehyde odor, comprising impregnating the textile with a formulation containing a methylol amide cross-linking agent for cellulose and a catalyst for effecting crosslinking of the cellulose by said crosslinking agent, and subjecting the resulting wet, impregnated textile, now containing free formaldehyde, to superheated steam at a temperature of about from 240° to 280° F. for about from 2 to 8 minutes to yield a sensitive cellulosic textile having a moisture content of about from 10 to three percent moisture, a formaldehyde odor which is imperceptible to the response of the olfactory capac-

ity of humans, and which is in a condition suitable for use in a post-cure durable-press process.

2. A method of sensitizing a cellulosic textile for use in the preparation of a post-cure durable-press product while simultaneously rendering the textile free of formaldehyde odor, comprising:

- a. impregnating the cellulosic textile with a formulation containing about from five to 20 percent of a cellulose crosslinking agent selected from the group consisting of dimethylol methyl carbamate, 10 dimethylol dihydroxyethyleneurea, dimethylol-4-methoxy-5,5-dimethylpropyleneurea, and bis-methoxymethyluron, and about from 0.3 to three percent of a zinc nitrate hexahydrate catalyst for effecting crosslinking of the cellulose by said crosslinking agent, and
- c. subjecting the resulting wet, impregnated textile, now containing free formaldehyde, to superheated steam at a temperature of about from 240° to 280° F. for about from 2 to 8 minutes to yield a sensitized cellulosic textile having a moisture content of 20

about from 10 to three percent moisture, a formaldehyde odor which is imperceptible to the response of the olfactory capacity of humans, and which is in a condition suitable for use in a post-cure durable-press process.

- 5
- 3. The method of claim 2 wherein the crosslinking agent is dimethylol methyl carbamate.
- 4. The method of claim 2 wherein the crosslinking agent is dimethylol dihydroxyethyleneurea.
- 5. The method of claim 2 wherein the crosslinking agent is dimethylol-4-methoxy-5,5-dimethylpropyleneurea.
- 6. The method of claim 2 wherein the crosslinking agent is bis-methoxymethyluron.
- 7. The product produced by the method of claim 1.
- 8. The product produced by the method of claim 2.
- 9. The product produced by the method of claim 3.
- 10. The product produced by the method of claim 4.
- 11. The product produced by the method of claim 5.
- 12. The product produced by the method of claim 6.

\* \* \* \* \*